

# United States Patent [19]

Burns

[11]

4,388,081

[45]

Jun. 14, 1983

[54] MOTOR FUEL

[75] Inventor: Lyle D. Burns, Bartlesville, Okla.

[73] Assignee: Phillips Petroleum Company,  
Bartlesville, Okla.

[21] Appl. No.: 393,238

[22] Filed: Jun. 29, 1982

[51] Int. Cl.<sup>3</sup> ..... C10L 1/18  
[52] U.S. Cl. ..... 44/78; 252/386  
[58] Field of Search ..... 252/386; 44/78;  
568/648

[56]

References Cited

U.S. PATENT DOCUMENTS

|           |        |                     |         |
|-----------|--------|---------------------|---------|
| 2,089,580 | 8/1937 | Schulze .....       | 44/9    |
| 3,270,497 | 9/1966 | Malick .....        | 60/35.4 |
| 3,642,911 | 2/1972 | Schulze .....       | 568/648 |
| 3,658,494 | 4/1972 | Dorer, Jr. .....    | 44/63   |
| 4,273,891 | 6/1981 | Pindar et al. ..... | 44/78   |
| 4,341,905 | 7/1982 | Strege .....        | 568/648 |

Primary Examiner—Charles F. Warren

Assistant Examiner—Y. Harris-Smith

[57]

ABSTRACT

Liquid hydrocarbon fuel compositions are provided containing antiknock quantities of ashless antiknock agents comprising phenoxyalcohols.

11 Claims, No Drawings

## MOTOR FUEL

This invention relates to liquid hydrocarbon fuel compositions having improved antiknock properties. In one of its aspects, this invention relates more particularly to liquid hydrocarbon fuel compositions intended for use in internal combustion engines containing novel and effective ashless antiknock agents. In accordance with a further aspect, this invention relates to liquid hydrocarbon compositions containing antiknock quantities of ashless antiknock agents selected from phenoxy alcohols and derivatives thereof.

Various antiknock agents have, heretofore, been suggested and employed for use in liquid hydrocarbon fuels, particularly in fuels employed in internal combustion engines. In such engines, it is highly desirable, from a stand point of economics that combustion of the fuel occurs at relatively high compression ratios. Such high compression ratios concomitantly necessitate the use of fuels having relatively high octane numbers to insure knock-free operation. Many antiknock agents have been proposed and/or used to improve the antiknock properties of hydrocarbon fuels used for internal combustion engines. In general, however, none of these antiknock additives have proved to be satisfactory in effectively raising the octane number of the fuel without also exhibiting other undesirable properties of varying importance. The phase-down of lead in gasoline as required by federal law and the banning of certain additives from use in unleaded gasoline has given impetus to continuation of a systematic study of the antiknock activity of ashless (non-metallic) compounds. The present invention is directed to the use of ashless (non-metallic) additives as antiknock agents for internal combustion fuels.

Accordingly, an object of this invention is to provide ashless hydrocarbon fuel compositions.

Another object of this invention is to provide ashless (non-metallic) antiknock additives for internal combustion engine fuels.

Another object of this invention is to provide hydrocarbon fuel compositions exhibiting improved antiknock properties.

Other objects, aspects, as well as the several advantages of the invention will be apparent to those skilled in the art upon reading the specification and the appended claims.

In accordance with the present invention, new and improved liquid hydrocarbon fuel compositions are provided containing an antiknock quantity of ashless (non-metallic) antiknock additives selected from phenoxyalcohols and derivatives thereof.

The antiknock additives of the invention are known and can be prepared by processes known in the art.

Specific examples of phenoxyalcohol ashless antiknock agents of the invention that can be used in internal combustion engine fuels include 2-phenoxyethanol, 2-(p-methylphenoxy)ethanol, 2-(p-t-butylphenoxy)ethanol, 2-(o-ethylphenoxy)ethanol, 1-phenoxy-2-propanol, 2-phenoxy-3-butanol, 1-(p-methylphenoxy)-2-propanol, 2-(p-methoxyphenoxy)ethanol, p-methoxybenzylalcohol and the like, and mixtures thereof, and structurally closely related compounds. These compounds have suitable solubility and volatility characteristics to permit their application as additives for hydrocarbon fuels.

The specific antiknock additives of the invention are highly suited for use in fuels in view of their ashless

characteristics. Naturally, the various compounds of the herein disclosed group do not possess exactly identical effectiveness, and the most advantageous concentration for each such compound will depend to some extent upon the particular compound used. Also, the minimum effective inhibitor concentration can vary somewhat according to the specific nature of the hydrocarbon composition to which it is added.

The amounts of the antiknock agents of the invention added to the hydrocarbon fuels will be sufficient to improve the antiknock properties of the fuel. In general, these novel antiknock additives are employed in amounts from about 0.5 to about 10 percent (5000 to 100,000 parts per million), preferably from about 1 to about 5 percent (10,000 to 50,000 parts per million), by weight of the total weight of the fuel composition.

The motor fuels or gasolines into which the invention additives are incorporated are conventional motor fuel distillates boiling in the range of about 70°-420° F. (21.1°-216° C.). Gasolines or automotive fuels to which the described additives perform the functions described herein include substantially all grades of gasoline presently being employed in automotive and internal combustion aircraft engines. Generally automotive and aircraft gasolines contain both straight run and cracked stock with or without alkylated hydrocarbons, reformed hydrocarbons, and the like. Such gasolines can be prepared from saturated hydrocarbons, e.g., straight run stocks, alkylation products, and the like, with or without gum inhibitors, detergents, corrosion inhibitors, solvents, emulsifiers, and the like. The motor fuels are unleaded and can contain other conventional fuel additives such as antioxidants and the like.

## SPECIFIC EXAMPLE

Six solutions with different concentrations of 2-phenoxy ethanol in clear (unleaded) FT-266 gasoline were prepared. The following table presents the characteristics of FT-266 gasoline.

## CHARACTERISTICS OF FT 266 TEST GASOLINE

| Description              | Unleaded premium pipeline base gasoline |
|--------------------------|-----------------------------------------|
| Designation              | FT-266                                  |
| Reid Vapor Pressure, psi | 5.7                                     |
| API Gravity @ 60° F.     | 60.3                                    |
| ASTM D-86 Distillation   |                                         |
| Vol % Evaporated         | Temp. °F.                               |
| IBP                      | 102                                     |
| 5                        | 142                                     |
| 10                       | 164                                     |
| 15                       | 178                                     |
| 20                       | 190                                     |
| 30                       | 210                                     |
| 40                       | 224                                     |
| 50                       | 235                                     |
| 60                       | 247                                     |
| 70                       | 264                                     |
| 80                       | 292                                     |
| 90                       | 335                                     |
| 95                       | 373                                     |
| EP                       | 431                                     |
| Research Octane Number   | 91.7                                    |
| Motor Octane Number      | 84.1                                    |

The gasoline was engine tested to determine its Research Octane Number (RON) according to ASTM D 2599-47. The increase in RON over the untreated fuel produced by the addition of the phenoxyalcohol compound is shown in the table. At 10 and 15% concentra-

tion two phases formed, and the upper fuel phase was used as the test sample.

| Additive Conc. (Vol. %) | RON Increase |
|-------------------------|--------------|
| 0                       | —            |
| 1.0                     | 0.6          |
| 2.0                     | 0.9          |
| 2.5                     | 0.8          |
| 5.0                     | 1.8          |
| 10 (Upper phase)        | 1.0          |

The results show the additive is effective as an octane improver.

The efficacy of the novel ashless antiknock compounds of the present invention for improving the anti-knock properties of liquid hydrocarbon fuels will be apparent from the foregoing example and comparative data. It will be understood that the novel ashless antiknock compounds of the present invention can be advantageously employed in any liquid hydrocarbon fuel composition which is suitable for use in a combustion engine regardless of the purpose for which the engine is designated.

I claim:

1. A fuel composition comprising a hydrocarbon suitable as a fuel for an internal combustion engine and an antiknock improving amount ranging from about 0.5 to about 10 weight percent of a phenoxyalcohol.

30

2. A composition according to claim 1 wherein said alcohol is 2-phenoxy ethanol.

3. A composition according to claim 1 wherein said amount ranges from about 1 to about 5 wt. %.

4. A composition according to claim 1 wherein said hydrocarbon is a distillate boiling in the range of about 70° F. to about 420° F.

5. A composition according to claim 1 wherein said hydrocarbon is unleaded gasoline containing 2-phenoxy ethanol.

6. A composition according to claim 5 wherein the amount of additive ranges from about 1 to about 5 wt. %.

7. A method for improving the antiknock properties of a motor fuel which comprises incorporating therein a small but effective amount ranging from about 0.5 to about 10 weight percent sufficient to impart reduced knocking tendencies to said motor fuel of an ashless antiknock additive comprising a phenoxyalcohol.

8. A method according to claim 7 wherein said motor fuel is unleaded and contains from about 1 to about 5 wt. % of the additive.

9. A method according to claim 7 wherein said motor fuel is unleaded gasoline.

10. A method according to claim 7 wherein said additive is 2-phenoxy ethanol.

11. A method according to claim 7 wherein said motor fuel contains from about 1 to about 5 wt. % of said alcohol.

\* \* \* \* \*

35

40

45

50

55

60

65